# EUROPEAN PATENT APPLICATION

(11) **EP 2 572 801 A1**
(43) Date of publication of application: **27.03.2013**
(21) Application number: 12185445.9
(22) Date of filing: 21.09.2012
(51) Int. Cl.: B05D 1/16, B32B 3/10, B32B 5/16, B32B 5/26, D06Q 1/10

(54) **Covering material and method for manufacturing such a covering material**

(30) Priority: 23.09.2011 BE 201100565
(71) Applicant: Flocart NV, 8560 Wevelgem (BE)
(72) Inventor: Vlieghe, Véronique, 8540 DEERLIJK (BE)
(74) Representative: Ostyn, Frans

(57) **Abstract**

The present invention relates to a covering material (1) comprising a carrier material (2) made of PVC-coated yarns, in which said covering material (1) comprises one or more flocked zones. By providing such zones on the covering material (1) made of PVC-coated yarns, the sitting comfort of the furniture which is covered with such a material will increase significantly.

## Description

The present invention relates to, on the one hand, a covering material comprising a carrier material made of PVC-coated yarns. On the other hand, the present invention relates to a method for manufacturing such a covering material.

The covering material according to the present invention can, inter alia, be used as covering for both outdoor furniture, such as for example beanbags, loungers, chairs and the like, and as covering for indoor furniture, without thereby wanting to limit the possible uses of the present invention.

Covering material which is made of PVC-coated yarn has already been commercially available for a considerable time. Due to its weatherproof nature and its resistance to tearing, such covering material is often used as self-supporting textile for outdoor furniture. Despite its many good properties, furniture which is covered with covering material made of PVC-coated yarn has the considerable drawback that the sitting comfort is inadequate.

It is therefore an object of the present invention to provide a covering material which, in use, will considerably improve the sitting comfort for the user.

The object of the invention is achieved by providing a covering material comprising a carrier material made of PVC-coated yarns, in which said covering material comprises one or more flocked zones. By providing such zones on the covering material made of PVC-coated yarns, the sitting comfort of the furniture which is covered with such a material will increase significantly.

Within the context of the present invention, the term "flocked zones" is understood to mean: zones in the covering material which comprise flock fibres which are secured to the carrier material by means of an adhesive connection. The flock fibres in question are preferably made of polyester, polyamide, viscose or cotton. The flock fibres are water- and dirt-repellent.

In a preferred embodiment of the covering material according to the invention, said zones comprise flock fibres which have a thickness in the range between 1 dTex and 5 dTex. In particular, said zones comprise flock fibres which have a length between 0.1 mm and 5 mm. In particular, said flock fibres are attached to the carrier material by means of an adhesive connection. The adhesive connection used is more particularly suitable to attach the flock fibres to PVC-coated yarns. The adhesive used is conductive, elastic and weather-proof.

According to a more particular embodiment of the covering material according to the invention, said carrier material is a woven, knitted or interwoven material.

Another object of the present invention relates to a method for manufacturing a covering material for furniture, which method comprises the following steps:
- supplying a carrier material made from PVC-coated yarn;
- applying a conductive adhesive layer to at least one zone of the carrier material supplied;
- applying flock fibres to the zones provided with adhesive by means of an electrostatic field;
- drying the carrier material.

The present invention will now be explained in more detail with reference to the following detailed description of some embodiments of the covering material according to the present invention. This description and these examples are solely intended to give an explanation and to indicate further advantages and particulars of these coverings according to the invention, and can therefore by no means be interpreted as a limitation of the area of application of the invention or of the patent rights defined in the claims.

In this detailed description, reference numerals are used to refer to the attached drawings, in which:
- *Fig. 1* *diagrammatically shows the covering material according to the invention;*
- *Fig. 2* *diagrammatically shows the method according to the invention.*

The covering material (1) according to the present invention and as illustrated diagrammatically in Fig. 1 is composed of a covering material (2), made of PVC-coated yarns. The covering material (2) may be a woven, knitted or interwoven material. Covering materials (1) made from such a material have already been commercially available for a considerable time, mainly as a self-supporting textile for outdoor furniture. However, a recurring complaint from consumers about these is that the sitting comfort of this known covering material is not satisfactory. According to the present invention, this problem is solved by providing the covering material (2) with one or more zones which comprise short fibres, so-called flock fibres (3). The presence of such "flocked" zones will significantly improve the sitting comfort of the furniture which is covered with such a material.

The flock fibres (3) used are made of polyester, polyamide, viscose or cotton, preferably have a thickness in the range from 1 dTex to 5 dTex, and a length of between 0.1 mm and 5 mm. The thinner the fibres (3), the softer the flocked surface is to the touch. It is important that the flock fibres (3) meet stringent criteria regarding colourfastness and rubbing fastness.

The way in which the covering material (1) according to the invention is formed is diagrammatically illustrated in Fig. 1. In this case, a carrier material (2) is provided with a conductive adhesive layer by means of a coating system (5) and template (6). Using an electrode (7), the flock fibres (3) are charged electrostatically and hurled at the conductive adhesive layer in this state. As a result of the charge in the fibre and the vibration of the carrier material, all the flock fibres (3) will stand upright. After the flock fibres (3) have been applied, the unit will be cured in a drying device (8) to form the flocked end product (1).

The covering material (1) according to the present invention is self-supporting, water-permeable, dirt-repellent and offers good sitting comfort. It is preferably used as covering for both outdoor furniture, such as for example beanbags, loungers, chairs and the like, and as covering for indoor furniture.

## Claims

1. Covering material (1) comprising a carrier material (2) made of PVC-coated yarns, **characterized in that** said covering material (1) comprises one or more flocked zones.

2. Covering material (1) according to Claim 1, **characterized in that** said zones comprise flock fibres (3) which have a thickness in the range between 1 dTex and 5 dTex.

3. Covering material (1) according to Claim 1 or 2, **characterized in that** said zones comprise flock fibres (3) which have a length between 0.1 mm and 5 mm.

4. Covering material (1) according to one of the preceding claims, **characterized in that** said carrier material (2) is a woven, knitted or interwoven material.

5. Covering material (1) according to one of the preceding claims, **characterized in that** said flock fibres (3) are made of polyester, polyamide, viscose or cotton.

6. Covering material (1) according to one of Claims 2 to 5, **characterized in that** said flock fibres (3) are attached to the carrier material by means of an adhesive connection.

7. Method for manufacturing a covering material (1) for furniture, **characterized in that** the method comprises the following steps:
- supplying a carrier material (2) made from PVC-coated yam;
- applying a conductive adhesive layer (4) to at least one zone of the carrier material (2) supplied;
- applying flock fibres (3) to the zones provided with adhesive by means of an electrostatic field;
- drying the carrier material (2).
